

# UNITED STATES PATENT OFFICE.

W. DEWEES WOOD, OF PITTSBURG, PENNSYLVANIA.

## PROCESS OF MANUFACTURING PLANISHED SHEET-IRON.

SPECIFICATION forming part of Letters Patent No. 291,260, dated January 1, 1884.

Application filed June 2, 1883. (No specimens).

*To all whom it may concern:*

Be it known that I, W. DEWEES WOOD, a citizen of the United States, residing at Pittsburgh, county of Allegheny, State of Pennsylvania, have invented or discovered a new and useful Improvement in the Process of Manufacturing Planished Sheet-Iron; and I do hereby declare the following to be a full, clear, concise, and exact description thereof.

10 My present invention relates to the manufacture of a kind of sheet-iron having a surface dark in color, but bright and glossy, and not liable to oxidation under the influence of the atmosphere or other usual surroundings 15 or conditions of use. Sheet-iron possessing these characteristics to a greater or less degree is already known in the art under the names of "Russia," "Imitation Russia," "Planished," &c., and processes of the manufacture of the same are described in sundry patents already granted to me. In the most 20 of these processes, and in fact, as I believe, in all in which by actual use any practical success has been attained, the broken-down iron 25 sheets have heretofore been subjected to the acid-sealing operation preliminary to the formation of a protective coating thereon; but several years of practical experience in the business have shown that, with such degree of 30 care as can ordinarily be secured from mill-operatives, some sheets will be passed and worked into final product, in which the acid will not be perfectly neutralized or the alkali will not be completely removed, and, as a result, 35 a small percentage of product is liable to go out, which will not be as free as is desired from liability to deterioration in use. My present process contemplates the entire disuse of the acid and alkali treatment and provides for 40 the formation or building up of an oxidized surface on each sheet and on each side of each sheet, over and above what is secured in the ordinary workings of the material employed, followed by the "reviving" or reconversion 45 of such oxidized surface back into metallic iron, or so nearly to that state or condition (sometimes called a "nascent" state or condition) that such "revived" or reconverted or nascent surface will enter readily into combination with or will freely and quickly com-

bine with an oxidizing agent supplied thereto in manner substantially as presently to be described, and thereby give an oxide surface adapted to protect the sheet, which oxide surface being fixed, as presently to be described, 55 is worked by heating and hammering or planishing till the desired product is secured.

In working my invention, I preferably use refined cast-iron, and, by known methods, get a bloom of a comparatively high degree of 60 purity. This I work down by ordinary forging or rolling operations to sheet form, of about No. 20 wire-gage, (more or less,) taking care throughout the operation to keep the material clear of free scale; but at the same time 65 I secure the formation on each face of each sheet of a fixed (as distinguished from a free or raised) black oxide coating, and on such coating I promote, so far as may be, the formation of a red oxide surface; and to this end 70 I give to each sheet, while undergoing the rolling operation, a free exposure on both sides to the atmosphere, changing or opening up the sheets frequently if rolled in doubles or packs, and also use water on the rolls with 75 considerable freedom, so that it shall run down on the sheets while passing through, or apply the water directly to the hot sheet by a brush or otherwise, but not in such amount as to cool them through or to interfere seriously 80 with their regular and uniform reduction by rolling. If any free scale is raised, it is to be carefully brushed off or otherwise removed. This method of treatment will give a fixed 85 black oxide coating on each surface of each sheet, and will form more or less red oxide on the top or surface of the black oxide. The sheets thus broken down, and with the black and red oxide coatings thereon, as thus described, are allowed to cool, and I then apply 90 to each surface of each sheet a coat or wash consisting of charcoal-dust, red oxide of iron, and suitable liquid—such as water or oil—made or mixed up thin, so as readily to be applied with a broom or other suitable implement, and by the use of which the wash is to be thoroughly rubbed in, or the rubbing action is to be kept up until the red oxide formed 95 on the sheet and the ingredients of the wash are well commingled, and are also distributed 100

with a good degree of uniformity over the surface of the sheet, on which they remain as a thin film or coating. This step in the process is directed especially to the building up or accumulation of a comparatively thick coating of oxide on each face of each sheet, and it differs from anything previously done to my knowledge, in this branch of the art, both in the intentional making of a red oxide on top of a black oxide by artificial means during the breaking-down operation, and also in adding thereto an additional quantity of artificially-applied red oxide, and, still further, in rubbing in the artificially-formed and applied red oxides, with reference to facilitating the operations next to be described. The pulverized charcoal is used chiefly to aid in the chemical operations subsequently taking place. In the preparation of this wash a finely pulverized or ground red oxide may be used; or, if not put in at first, the repeated washings and rubbing of successive sheets, and the redipping of the brush or broom or other implement into the liquid will soon so impregnate or charge the wash with the red oxide taken from the sheets that it will answer the purpose in view. If the work thus far is well and carefully done, enough red oxide will be formed on the sheets for the purpose of this invention. The sheets are then matched up in packs—say of from three to six sheets, more or less, according to the gage of product desired, and are then heated in an ordinary or any suitable sheet-reheating furnace, and rolled, again heated and rolled in the manner common in doing such work, until the sheets are brought down to or approximately to the desired gage. The first of these heatings should be to or about a bright red, and subsequent ones to a lower temperature—say a dull red. During the rolling operations the sheets are to be opened up from time to time, to see that they are clear of dirt and free scale and do not stick, &c., in the process of rolling. The sheets, then being cold, are again rubbed as before, separately and on both sides with a wash of red oxide and water, or with the same wash as previously used, and while they are still wet therefrom I throw or sprinkle onto each wet surface a coating of charcoal-dust, preferably somewhat coarse, till it is well covered at every point—say, thick enough to cover the surface of the sheet from sight; or it may be thicker still without danger of injurious results. The sheets, as fast as they are thus coated, are piled one on top of another, till a package is formed of from, say, twenty to one hundred sheets, more or less; but the sheets, when dry, may be thus built up into a package, with intermediate layers of charcoal, if so desired; but the work can be done with greater ease and facility when the sheets are wet. Such package is then charged into a chamber or retort of iron or clay or other suitable material, which is then closed up air-tight and subjected to external heat—about a white heat—for from, say, four to eight hours. (more or less,) or

till the fixed oxide on the surfaces of the sheets has, by the action of the carbon of the charcoal, become revived, or reconverted into metallic iron, or brought so near to the condition of metallic iron that it is just ready to come, or on the point of coming, to that condition, and it may then be termed "nascent" iron. The package is then removed with the sheets still at a high temperature. Immediately thereon, and before any injurious effects are produced by atmospheric exposure, I quickly remove the refuse material—such as ashes, unconsumed charcoal, &c.—from the face of each sheet, and simultaneously or immediately after supply an oxidizing agent to each revived, reconverted, or nascent surface, so as to form a black or magnetic oxide thereon, and before the internal heat of the sheet or the external air can act to "raise" or free the oxide so formed I chill or cool the sheet to such a degree as to arrest further chemical action. In this way I get on each surface of each sheet a black oxide of uniform quality and thickness, and fix it so that the sheet is then in condition for further working. In doing this work various devices may be employed, and the right to patent such devices separately, so far as they may involve invention, is hereby reserved; but, that the present invention may be the better understood, I will describe one way of doing it, which I particularly claim as of my own invention. Over and along each surface of each sheet, as soon as it is uncovered or exposed, I play a series of jets of superheated steam under a high pressure, the jets being of such size and so close together, and striking the sheet at such angle, that they will thoroughly blow off the waste material remaining on the sheet, and at the same time will furnish to the hot sheet such amount of oxygen (by decomposition) as to convert the revived or nascent iron of the surface, or will form thereon a black or magnetic oxide over its whole surface, and practically uniform in thickness. This I follow quickly by an application through the use of a sponge, mop, brush, or otherwise, of cold water, in such manner and amount as to cool the sheet sufficiently to arrest further chemical action, either from the internal heat of the sheet or from the external air, and by so doing I fix the oxide so formed as against any tendency to raise or form a free scale; but other suitable means of doing the same work may be employed. Ordinarily the sheets will still be quite warm, and they may then be hammered to take out any irregularities—such, for example, as result from buckling in cooling. They are then matched up into packs as before, charged into a sheet-reheating furnace, and raised, say, to a fish-worm red, then hammered thoroughly all over by planishing-hammers in the manner already known in the art, and this reheating and planishing operation is repeated one, two, three, or more times, until the desired surface is obtained, which is a brilliant blue polished surface, superior in all respects to the best Russia.

I claim herein as my invention—

1. In the manufacture of planished sheet-iron, the improved method of preparing broken-down iron sheets for subsequent working, which consists in coating the same with a wash of red oxide of iron, carbon, and water, or other suitable liquid, substantially as set forth.
2. In the manufacture of planished sheet-iron, the improved method of preparing the broken-down iron sheets for subsequent working, which consists in rubbing up the red oxide formed on the sheets while being rolled and simultaneously applying and rubbing in an artificial wash of red oxide, carbon, and suitable liquid, substantially as set forth.
3. In the manufacture of planished sheet-iron, the improved method of preparing the sheets for treatment in a closed retort or chamber, which consists in coating the same with artificially-applied red oxide and pulverized carbon, substantially as set forth.
4. In the manufacture of planished sheet-iron, the improved method of treating the hot sheets as they come from the retort, which consists in quickly removing the waste material therein, reoxidizing the revived or nascent surface while still hot, and immediately cooling the sheet by artificial means, substantially as set forth.
5. The improved method of cleaning and simultaneously reoxidizing the revived or nascent surface of a sheet previously coated with an oxide and deoxidized in a closed retort or

chamber, which consists in causing a series of jets of superheated steam under high pressure to discharge or blow on and along the exposed surface of such sheet while still hot from the retort or chamber, substantially as set forth.

6. In the manufacture of planished sheet-iron, the improved method of treatment embracing the following steps: first, subjecting the unscaled sheets in packs, with intervening layers or coatings of carbon, to the action of a high heat in a close chamber or retort; second, causing a series of steam-jets to discharge or blow on and along the exposed surface of each sheet while still hot from the retort or chamber; and, third, arresting further chemical action by artificial means, substantially as set forth.

7. The improvement in the process of making planished sheet-iron, which consists in artificially promoting thereon, substantially as described, the formation of an oxide surface, reviving such oxide surface, reoxidizing such revived or nascent surface, and fixing the oxide so formed, with intermediate heating and rolling and final heating and planishing, substantially as hereinbefore set forth.

In testimony whereof I have hereunto set my hand.

W. DEWEES WOOD.

Witnesses:

R. H. WHITTLESEY,  
C. M. CLARKE.